

## UNITED STATES PATENT OFFICE

DONALD W. RANDOLPH, OF FLINT, MICHIGAN, ASSIGNOR TO A C SPARK PLUG COMPANY, OF FLINT, MICHIGAN, A COMPANY OF MICHIGAN

## PROCESS OF MAKING ALLOYS

No Drawing.

Application filed May 26, 1932. Serial No. 613,767.

This is a continuation in part of my prior application S. N. 520,704, filed March 6, 1931.

This invention relates to a process of making alloys containing low melting point 5 metals such as barium. Barium has a low work function—in other words, it gives off electrons easily,—so that alloys containing it are particularly desirable for use in spark plug electrodes to give a low and uniform 10 sparking voltage, and in the cathodes of vacuum tubes and the like because of the profuse emission of electrons with small current consumption.

Owing to the fact that barium has a low 15 melting point and is readily oxidized considerable difficulty has been experienced in the past in alloying it with suitable base metals. By following my method it is possible to produce at will alloys containing any 20 desired barium content within the limits disclosed. I have chosen nickel as the base metal for the reason that it alloys well with barium and possesses in itself properties valuable for use in spark plug and vacuum tube elec- 25 trodes. The closely related metal, cobalt, also possesses some advantages as a base for the alloy as will be pointed out.

In preparing the alloy, nickel is melted, 30 preferably in a high frequency induction furnace, although this is not essential. The melt is preferably held at a temperature a little above the melting point, and to the melt is preferably added a proportion of manganese, for example, 2 parts of manganese to 98 parts 35 of nickel. The manganese performs its usual functions as a deoxidizer. The temperature of the melt is then preferably raised from a little above the melting point, which is about 2620° F. to approximately 2800° F. to 2850° 40 F. and is held at that temperature for from 2 to 5 minutes to insure thorough alloying of the elements. I prefer the shorter period. Next  $\frac{1}{10}$  of 1% magnesium is added, this addition being for the purpose of rendering the 45 alloy more ductile. The melt is then held at the same temperature for one minute, to insure thorough admixture of the magnesium with the other constituents.

The barium is furnished in blocks or bars 50 and I have found it essential to protect it

from moisture and oxidation after cutting it off from the mass and before introducing it into the melt. I have had the best success by immediately dipping the severed portion in quick drying pyroxylin lacquer such as is used 55 on automobile bodies. The lacquer completely excludes air and moisture. The barium is then wrapped in nickel foil, or inserted in a tin box provided with a practically air tight closure and is immersed in the melt. This 60 may best be done by wrapping the end of a nickel wire about the package and plunging it beneath the surface of the molten metal, using the wire as a handle. The barium is added in amount equalling about 2% of the melt, 65 and is added one minute after the addition of the magnesium. After the addition of the barium, the melt is permitted to stand for about 30 seconds and is then poured into a warm steel mold. 250° F. is a suitable mold 70 temperature.

By adhering to the steps outlined I am able to consistently produce alloys containing as high as .17% barium. I have also found that the time schedule is equally satisfactory for 75 2½ lb. melts and for 250 lb. melts, although it might be thought that a longer alloying time would be necessary with the larger amount of metal.

I regard as the most important step of the 80 method, the maintaining of the temperature of the metal somewhat above the melting point, for example, in the neighborhood of 2800° F. to 2850° F. and casting of the ingot within a very short period, i. e. thirty seconds, 85 after the addition of the barium. If the melt were allowed to stand for many minutes after the addition of the barium practically none of the barium would be found to be present in the cast ingot.

In the larger melts I have found it desirable to add the barium in lumps not exceeding 90 100 grams each, adding two or more of the lumps to produce the desired constituency.

If the melt is poured too soon after the addition of the barium, a non-uniform composition is obtained, part of the barium separating out without alloying.

I have in some cases employed cobalt in 100

place of nickel. Cobalt seems to increase thermionic emission. I have made by the described methods alloys differing from that detailed, by the substitution of cobalt for 5 80% of the nickel. I have found, however, that the addition of more than 25% cobalt produces an alloy that corrodes rapidly when used as a spark plug electrode. I have used the term "nickel-cobalt metal" to designate 10 this preferred group of base metals.

I have also made an alloy of this type by first making a sub-alloy of 45% nickel and 55% manganese, this composition having the lowest boiling point of any combination of 15 nickel and manganese. To this sub-alloy I have added barium, and the resulting alloy I have added to nickel to form the desired composition, but this modification has produced no better results than the preferred 20 procedure.

I have found it desirable in some cases to add chromium to the alloy. In the case of spark plug electrodes the addition of chromium reduces corrosion, and for this purpose from 1 to 20% may be added. An alloy 25 of this type containing chromium has also proven of special value for vacuum tube filaments. I have described and claimed in my copending application Serial No. 520,703 filed 30 March 6, 1931, a nickel-barium-chromium alloy suitable for these purposes.

The chromium is preferably added to the alloy before the barium, the procedure being otherwise that given above.

35 I claim:

1. The method of producing an alloy of nickel and barium which consists in melting the nickel metal and maintaining it at a temperature of approximately 2800° F. to 2850° 40 F., coating or covering the barium to render it impervious to air and moisture, immersing the barium beneath the surface of the melt, and maintaining it at the said temperature for a short period to insure thorough 45 alloying, and immediately pouring the resulting alloy.

2. The method of producing an alloy of nickel and barium which consists in melting the nickel and maintaining it at a temperature of approximately 2800° F. to 2850° F., coating or covering the barium to render it impervious to air and moisture and permit its immersion in the melt, immersing the barium beneath the surface of the melt and 55 maintaining it at the said temperature for a short time, on the order of 30 seconds, to insure thorough alloying, and immediately pouring the resulting alloy.

3. The method of producing an alloy of 60 nickel and barium which consists in melting the nickel, adding suitable amounts of a de-oxidizing agent, maintaining the melt at a temperature of approximately 2800° F., coat-

ing or covering a quantity of barium to render it impervious to air and moisture and to temporarily protect it from the heat of the melt to permit of its immersion therein, inserting the barium thus prepared beneath the surface of the melt and maintaining it at such temperature for a short time, on the order of thirty seconds, to insure thorough alloying, and immediately pouring the resulting 70 alloy into a suitable mold.

4. The method of producing an alloy of nickel and barium, which consists in melting the nickel and maintaining it at a temperature of approximately 2800° F. to 2850° F., providing a quantity of barium with a consumable coating to exclude air and moisture, and with an outside fusible metallic covering, inserting the barium thus prepared beneath the surface of the melt and maintaining it at such a temperature for a short time to insure 75 thorough alloying, and immediately pouring the alloy into a suitable mold.

5. The method of producing an alloy of nickel and barium which consists in melting the nickel metal, maintaining it at a temperature but slightly above melting, adding a small percentage of a suitable deoxidizing agent, raising the temperature to approximately 2800° F. to 2850° F. and holding it there for a few minutes to insure thorough alloying, adding a small proportion of magnesium to render the alloy ductile, holding the melt at said temperature for approximately one minute, coating or covering a 80 quantity of barium to render it impervious to air and moisture and to temporarily protect it from the heat of the melt to permit of its immersion therein, inserting the barium thus prepared beneath the surface of the melt and maintaining it at said temperature for 85 a short time, on the order of thirty seconds, to insure thorough alloying, and immediately pouring the alloy.

6. The method of producing an alloy of nickel and barium, which consists in melting the nickel, maintaining it at a temperature but slightly above melting, adding a small percentage of manganese, raising the temperature to approximately 2800° F. to 2850°

F. and holding it there for from two to five 100 minutes to insure thorough alloying, adding a small proportion of magnesium to render the alloy ductile, holding the melt at said temperature for approximately one minute, providing a quantity of barium with a consumable coating to exclude air and moisture, and with a fusible metal covering, inserting the barium thus prepared beneath the surface of the melt and maintaining it at said temperature for a short time, on the order of 105 thirty seconds, to insure thorough alloying and immediately pouring the alloy.

DONALD W. RANDOLPH.